

# UNITED STATES PATENT OFFICE.

JANE MOORE, OF CAMBRIDGE, MASSACHUSETTS.

## LEATHER-DRESSING.

SPECIFICATION forming part of Letters Patent No. 572,489, dated December 1, 1896.

Application filed May 14, 1896. Serial No. 591,490. (No specimens.)

*To all whom it may concern:*

Be it known that I, JANE MOORE, of Cambridge, county of Middlesex, State of Massachusetts, have invented an Improvement in 5 Leather-Dressing, of which the following is a specification.

My invention relates to a compound especially intended for dressing leather, and particularly patent or enameled leather.

10 In the manufacture of patent-leather the leather is very apt to be weakened in the baking-oven and the fiber thereof rendered weak and comparatively lifeless, and therefore it is necessary that the leather shall receive not only a certain amount of strength and permanency from the dressing, but the dressing should be of such a character as to give a degree of nourishment and pliability to the leather as well as to suitably improve 15 and strengthen the enamel, rendering the latter tough, brilliant, and pliable without liability to crack or become otherwise injured.

It is the object of my invention to meet all these requirements in an improved dressing, 20 consisting, preferably, of the following ingredients compounded substantially in the proportions herein set forth, although I do not intend to limit my invention precisely to these proportions: one gallon paraffin-oil, four 25 ounces pure beeswax, one-half ounce pulverized Spanish licorice, one-eighth ounce Pará rubber-gum, and one-eighth ounce gutta-percha.

I prepare the compound dressing in substantially the above proportions, as follows: 30 The paraffin-oil or other vehicle, if preferred, and the wax and Spanish licorice are mixed and kept at a boiling-point until the wax is entirely dissolved. The rubber and gutta-percha, which have been previously cut up by suitable means, as, preferably, by a small amount of petroleum-oil, (two ounces,) to which, preferably, about four grains of borax has been added as an antiseptic, are then 35 mixed with a suitable portion of the paraffin-oil or other vehicle until wholly dissolved. As the previously-boiled wax and licorice mixture cools, the latter rubber and gutta-percha mixture is stirred in thoroughly until 40 the entire dressing compound has cooled. The dressing is then properly strained.

The compound as thus prepared is espe-

cially intended as a manufacturers' dressing for use in the preparation of patent-leather or enameled-leather stock.

When this dressing is to be used as an outer dressing for the finished articles into which the leather is manufactured, I add, preferably, about three ounces of ivory-black to the compound when at the boiling-point, and when cool whip to a cream.

The ordinary dressings for patent-leather which are now in common use invariably contain some special drying ingredient. It is one object of my invention to avoid this, for 65 the reason that any specific drying ingredient is particularly injurious to patent-leather.

The enemy of patent-leather is the drying effect of the atmosphere, and therefore the leather needs a strengthening and softening 70 nourishment to prevent it from hardening and cracking. Beeswax contains the essential nourishment which the peculiarly dry and tender leather forming the body of patent-leather requires. The paraffin-oil acts 75 preferably as a carrier, as this oil is not over-hardening, being only slowly volatile, and also as it never becomes rancid it has no tendency to disintegrate and dissolve the enamel or to render the same dull, as would otherwise be 80 the case. The rubber is introduced for the purpose of giving elasticity and permanence to the leather and enamel, more particularly to the latter, and also preserves and increases the shine. The gutta-percha is particularly 85

useful in preventing the chipping off of the enamel, rendering the same tough and integral with the leather, and, in fact, giving to both the leather and the enamel unusual strength. The Spanish licorice is found to be 90 of extreme value in my compound, inasmuch as it gives the enamel a remarkably superior finish, not only in brilliancy and permanency of shine to the surface, but it also gives the enamel a peculiar smoothness and fine quality, so that the enamel is entirely without liability to stick to the machinery or to itself when passed through the machinery or when doubled over on itself. I consider the softening and brilliancy given to the enamel by 95 100 this feature of my invention as of superior importance.

A further general quality of my compound dressing is that it permeates and supports

the fibers of the leather, rendering the same non-absorbent and preventing the same from becoming overdrawing and from absorbing the ammonia and other deleterious matters from the feet.

5 What I claim as my invention, and desire to secure by Letters Patent, is—

1. The herein-described dressing, consisting of a compound of rubber, gutta-percha, 10 Spanish licorice, and a vehicle, substantially as described.

2. The herein-described dressing, consisting of a compound of wax, rubber, Spanish licorice and a vehicle, substantially as de- 15 scribed.

3. The herein-described dressing, consisting of a compound of wax, gutta-percha, Span-

ish licorice, and a vehicle, substantially as described.

4. The herein-described dressing, consisting of a compound of rubber, Spanish licorice, and a vehicle, substantially as described.

5. The herein-described dressing, consisting of a compound of wax, rubber, gutta-percha, Spanish licorice, and paraffin-oil, sub- 25 stantially as described.

In testimony whereof I have signed my name to this specification in the presence of two subscribing witnesses.

JANE MOORE.

Witnesses:

LAURA T. MANIX,

THOMAS J. DRUMMOND.